

[54] EXTRUSION DIE

[75] Inventor: **Friedrich Franz Xaver Heitzinger**,  
Lechaschau, Austria[73] Assignee: **Schwarzkopf Development  
Corporation**, New York, N.Y.[22] Filed: **Jan. 29, 1971**[21] Appl. No.: **111,136**

## [30] Foreign Application Priority Data

Feb. 2, 1970 Austria ..... 906/70

[52] U.S. Cl. .... **29/182.5**, 72/467, 75/206[51] Int. Cl. .... **B22f 5/00**

[58] Field of Search ..... 75/206; 29/182.5; 72/467

## [56] References Cited

## UNITED STATES PATENTS

2,949,358 8/1960 Alexander et al. .... 75/206  
3,271,142 9/1966 Hammond et al. .... 75/206  
3,475,159 10/1969 Hansen ..... 75/206

2,798,808 7/1957 Iredell et al. .... 75/206

## FOREIGN PATENTS OR APPLICATIONS

1,242,810 6/1967 Germany

## OTHER PUBLICATIONS

Goetzel, Treatise on Powder Metallurgy, 1950, Vol II  
pp. 685, TN695 60, Interscience Pub.Harwood, The Metal Molybdenum, ASM, 1958, pp.  
25-27, 29 & 30, TN799 M7U55.

Primary Examiner—Leland A. Sebastian

Assistant Examiner—B. Hunt

Attorney, Agent, or Firm—Morgan, Finnegan, Durham  
& Pine

## [57] ABSTRACT

This invention relates to extrusion dies useful for processing both non-ferrous metals and alloy steels, the dies being made of a predominant amount of molybdenum or tungsten, the remainder being zirconia.

**5 Claims, No Drawings**

1  
EXTRUSION DIE

Extrusion dies for the processing of various metals including non-ferrous metals and alloy steels, are well-known. Conventional dies of this type are made from stellites and high temperature steels. Some dies are also made from such oxide materials as zirconia. However, these materials have been found to be disadvantageous. They are difficult to work and because of their brittleness they develop cracks during operation. Consequently, their useful life is quite short.

By means of this invention it is possible to prepare extrusion dies having sufficient ductility and an outstanding resistance to cracking. The dies of this invention contain from 85 to 98 percent by volume of molybdenum or tungsten with the remainder being a zirconia phase. Preferably, the molybdenum or tungsten phase will be in excess from 85 to 95 percent by volume of the composition.

Mixtures of molybdenum and tungsten or alloys of 20 molybdenum and tungsten can also be employed in place of molybdenum or tungsten alone.

The zirconia phase is preferably stabilized by a zirconia stabilizing oxide. Such zirconia stabilizing oxides include calcium oxide, magnesium oxide and oxides of cerium and yttrium. Where employed, the stabilizing oxides are present in an amount of up to about 30 percent by volume of the zirconia phase.

The dies of this invention are prepared by conventional powder metallurgical techniques. The powdered materials employed preferably have a particle size of from 0.1 to 30 microns. The powdered materials are mixed together and then compressed to form compacts having approximately the desired final shape. The pressures employed can range from 15,000 to 80,000 p.s.i. The pressed compacts are then sintered in a reducing or inert atmosphere as, for example, in a hydrogen atmosphere or in an atmosphere of an inert gas such as helium or argon, or the like. The sintering temperature should be from about 1,700° to 2,200° C. If desired, 40 pressure can be maintained during sintering, although it is not required. Sintering time will depend upon the size and thickness of the compact but will generally range from about 2 to about 30 hours. After sintering

## 2

and cooling, preferably while the inert or reducing atmosphere is maintained, the desired final form of the die is obtained by machining to the final shape. More complex shapes can be made by spark erosion.

- 5 The final die produced in accordance with this invention has a long service life and can be successfully used for the extrusion of steel or non-ferrous metals. Furthermore, the nature of the die of this invention generally eliminates the tendency of welding of the die to the 10 extruded material. Consequently, it is generally possible, when using the dies of this invention, to dispense with the use of lubricants during extrusion without risking the likelihood of particles of extruded metal sticking to the die.
- 15 A suitable extrusion die can be manufactured by mixing 94.5 weight per cent of fine molybdenum powder having a particle size of 4 microns, 5.1 percent by weight of powdered zirconia having a particle size of 1 and 0.4 weight per cent of magnesium oxide (magnesia) having a particle size of 0.1. Thereafter, the mixture is pressed to form a compact by application of pressure using conventional powder metallurgical techniques of 40,000 p.s.i. The pressed compacts are then sintered at 2,000° C. for 8 hours in a hydrogen atmosphere. 25 They are thereafter permitted to cool in hydrogen and finally the final desired form of the die is obtained by machining the sintered compacts.

What is claimed is:

1. An extrusion die for the processing of metallic materials, said extrusion die consisting essentially in excess of 85 percent by volume but not more than 95 percent by volume of molybdenum or tungsten, the remainder being a zirconia phase.
- 30 2. An extrusion die as in claim 1 wherein the zirconia phase contains zirconia and one or more stabilizers for the zirconia.
- 35 3. An extrusion die as in claim 1 wherein the stabilizer for the zirconia phase is selected from among the oxides of calcium, magnesium, cerium and yttrium.
- 40 4. An extrusion die as in claim 1 consisting essentially of molybdenum and zirconia.
5. An extrusion die as in claim 1 consisting essentially of tungsten and zirconia.

\* \* \* \* \*

45

50

55

60

65